

Jan. 19, 1926.

1,570,420

V. YNGVE

ELECTRICAL CONTACT MAKER AND BREAKER

Filed June 20, 1924



Inventor  
Victor Yngve

by Panerai  
his Atty

## UNITED STATES PATENT OFFICE.

VICTOR YNGVE, OF SOUTH ORANGE, NEW JERSEY, ASSIGNOR TO MANHATTAN ELECTRICAL SUPPLY COMPANY, INCORPORATED, OF NEW YORK, N. Y., A CORPORATION OF MASSACHUSETTS.

## ELECTRICAL CONTACT MAKER AND BREAKER.

Application filed June 20, 1924. Serial No. 721,353.

*To all whom it may concern:*

Be it known that I, VICTOR YNGVE, a citizen of the United States, residing at South Orange, in the county of Essex and State of New Jersey, United States of America, have invented certain new and useful Improvements in Electrical Contact Makers and Breakers, of which the following is a specification.

10 This invention relates to improvements in electrical contact makers and breakers, and more particularly to a new commutator adapted for use in circuits of electrical motors and the like.

15 In accordance with the present invention, the contact points of a circuit maker and breaker or the contacting surface of a commutator, is covered with a thin coating of metallic chromium. Preferably, the working surfaces of the contact points or commutators of copper, bronze or the like, are electroplated with chromium, best results being obtained by using Sargent's solution of 245 g./L chromic acid and 3 g./L chromium sulfate, and a current density of 13.4 amp./sq. dm. (125 amp. sq. ft.), using a chromium anode.

20 Chromium is exceedingly hard and holds a bright, silver-like lustre almost indefinitely. Furthermore, chromium resists corrosion. Owing to its resistance to corrosion and its hardness, a chromium surface is preferable, for the present purposes, to a copper surface. While the electrical con-

ductivity of chromium is only about one-fifth that of copper, this is not an impediment to its use in commutators or the like, because, in accordance with the present invention, the circuit controller is coated with a very thin layer (e. g., .005 of an inch) of a 40 metallic chromium. The relatively high resistance offered by this thin layer is negligible as compared with the advantages obtained from its resistance to wear and corrosion.

45 The drawing illustrates in vertical cross-section a commutator, the contacting surface of which is electroplated with metallic chromium.

50 What I claim is:

1. An electrical circuit controller coated with metallic chromium.
2. An electrical circuit maker and breaker, electroplated with a coating of metallic chromium.
3. An electrical circuit maker and breaker, the contacting surface of which is electroplated with a coating of metallic chromium of a thickness of about .005 of an inch.
4. A commutator having on its contacting surface an electrolytically deposited layer of chromium of a thickness of about .005 of an inch.

55 In testimony whereof, I have signed my name to this specification this 17th day of June, 1924.

VICTOR YNGVE.